

July 16, 1946.

C. F. ALBAN ET AL

2,403,895

THERMOSTATIC METAL

Filed Feb. 28, 1942

2 Sheets-Sheet 1

COEFFICIENTS OF EXPANSION  
EXPANSIVITY OF THE Cu. Mn. ALLOYS



Fig. 1

INVENTORS  
Clarence F. Alban  
BY  
Stanley R. Hood  
Barnes, Kisselle, Laughlin & Raisch  
Attorneys.

July 16, 1946.

C. F. ALBAN ET AL

2,403,895

THERMOSTATIC METAL

Filed Feb. 28, 1942

2 Sheets-Sheet 2

Fig. 2



Fig. 3

INVENTORS  
Clarence F. Alban  
Stanley R. Hood

BY

Barnes, Kisselle, Laughlin & Price  
Attorneys.

## UNITED STATES PATENT OFFICE

2,403,895

## THERMOSTATIC METAL

Clarence F. Alban, Pontiac, and Stanley R. Hood,  
Birmingham, Mich., assignors to W. M. Chace  
Company, Detroit, Mich., a corporation of  
Michigan

Application February 28, 1942, Serial No. 432,832

2 Claims. (Cl. 297—15)

1

This invention relates to thermostatic metal. This application is a continuation-in-part of our application Serial No. 315,130, filed January 22, 1940, now abandoned.

It is a common expedient in temperature responsive mechanisms and controls to utilize the difference in expansion of two metals or alloys to effect mechanical movement. The mechanical movement is usually obtained by using one metal having a high coefficient of expansion and another metal having a low coefficient of expansion which are either fused together to form thermostatic bimetal or mechanically arranged as, for example, a rod within a tube. The degree of movement obtained and the amount of work produced depends in general on three factors: the strength of the materials used, the temperature change, and the difference in expansion coefficients of the two metals.

The following metals and alloys having high coefficients of expansion are commonly used in temperature responsive mechanisms and controls: copper, brass (60% copper, 40% zinc) and iron-nickel alloys to which may be added chromium, for example, an alloy containing 22% nickel, 3% chromium, 75% iron. Up to the present no alloy has been developed which has both an expansion rate higher than a 60-40 brass and good strength characteristics at temperatures as high as 500° C. For a low expansive element iron-nickel alloys containing between 35% and 50% nickel are commonly used. Invar (36% nickel, 64% iron) is one such alloy commonly used for the low expansive element. The low expansive element can also be made from an alloy of 17% chromium, 4% aluminum, balance iron.

It is an object of this invention to produce a laminated thermostatic metal which has a higher electrical resistivity and which will produce a remarkably higher strain energy per degree temperature difference than any other known thermostatic metal.

This invention also contemplates a laminated thermostatic metal having an appreciably higher deflection rate than any other known thermostatic metal.

This object has been achieved by utilizing a binary alloy of manganese and copper or a ternary alloy of manganese, copper and one of the iron group metals, as the high expanding lamina of the thermostatic metal. Manganese, both commercially pure manganese and electrolytic manganese, has properties which make it desirable as the high expanding lamina of thermo-

static metal, such as a high melting point, a high coefficient of expansion and high strength at high temperatures, but since manganese is brittle it alone cannot be used for the high expanding lamina of thermostatic metal. Because of this manganese is alloyed with copper which produces a ductile alloy having a high melting point, high strength at high temperatures and a remarkably higher coefficient of expansion than either pure manganese or copper and a remarkably higher electrical resistivity.

According to Mechanical Engineers' Handbook by Lionel S. Marks, fourth edition, 1941, page 624, manganese has a linear coefficient of thermal expansion per degree F. at about 70° F. of  $12.8 \times 10^{-6}$ , nickel  $7.2 \times 10^{-6}$ , and copper  $9.12 \times 10^{-6}$ . This remarkable increase in thermal expansion of the alloy in contrast to manganese is remarkably demonstrated, by way of example, if one considers the coefficient of expansion of an alloy consisting of 72% manganese, 18% copper, and 10% nickel. According to the law of mixtures, one would expect a low linear coefficient of expansion for this alloy of  $11.57 \times 10^{-6}$  per degree F. at about 70° F. Actually one gets the remarkably high linear coefficient of expansion of  $15.5 \times 10^{-6}$ . Because of this property of the manganese alloy, the thermostatic metal, which is the subject of this invention, has a remarkably high deflection rate.

In fabricating the high expanding lamina the best analysis having the highest strength, highest expansion rate and highest electrical resistivity is a ternary alloy consisting of 72% manganese, 18% copper and 10% nickel. Although the above is the preferred analysis, other excellent alloys can be obtained for use as the high expanding lamina wherein the manganese ranges from 60% to 85% of the alloy by weight, wherein the copper ranges from 10% to 35% by weight of the alloy, and wherein the nickel ranges from 5% to 30% by weight of the alloy. Although the above are the preferred ranges of the constituents of the alloy, these ranges can be widened somewhat to include other analyses which produce a material much better suited as the high expanding lamina of thermostatic metal than other known materials. In this enlarged range the constituents by weight would comprise the following percentages of the alloy: manganese 15% to 95%, copper 85% to 5%, nickel 0% to 30%. Cobalt or iron can be substituted wholly or in part for nickel in the ranges above specified. However, nickel is preferred over either cobalt or iron. Nickel when alloyed with copper

and manganese raises the elastic limit of the alloy and improves the physical properties in general of the alloy. The nickel also gives the alloy stability, that is, causes the alloy upon cooling to travel along the same curve that it traverses while being heated. In other words, nickel causes the alloy when its expansion and contraction characteristics, due to thermal change, are plotted on a graph, to travel along the same curve upon a fall in temperature that it traveled upon a corresponding rise in temperature.

Manganese having a purity of 99.98% can be produced electrolytically. So-called commercially pure manganese usually contains about 3% to 5% of impurities, such as iron, carbon, aluminum and silicon. In the above analyses it is preferred to use electrolytically pure manganese throughout the entire range. However, commercially pure manganese can be used up to a point at which the commercially pure manganese approximates about 35% of the alloy. Where the manganese comprises more than 35% of the alloy, then to avoid brittleness it is essential that all amounts of manganese over about 35% of the alloy should be electrolytically pure manganese.

The following expansion data is characteristic of the following alloys:

| Temp.,<br>° C. | $\alpha \times 10^{-6}$<br>23% Mn, 4%<br>Fe, balance<br>Cu | $\alpha \times 10^{-6}$<br>27% Mn, 4%<br>Fe, balance<br>Cu | $\alpha \times 10^{-6}$<br>32% Mn, 5%<br>Ni, 5% Fe,<br>balance Cu | $\alpha \times 10^{-6}$<br>9% Mn, 5%<br>Ni, balance<br>Cu |
|----------------|------------------------------------------------------------|------------------------------------------------------------|-------------------------------------------------------------------|-----------------------------------------------------------|
| 100            | 20.7                                                       | 21.3                                                       | 21.3                                                              | 18.7                                                      |
| 200            | 22.0                                                       | 22.5                                                       | 22.9                                                              | 19.2                                                      |
| 300            | 22.4                                                       | 23.0                                                       | 24.3                                                              | 20.1                                                      |
| 400            | 23.4                                                       | 23.9                                                       | 25.2                                                              | 22.2                                                      |

Expansion data and representative resistance data is herewith set forth of the below specified alloys:

| Alloy   | Temperature range<br>20°-450° coefficient<br>of expansion cm. per<br>cm. per degree C. | Resistance<br>in ohms per<br>circular mil<br>foot at 20° C. |
|---------|----------------------------------------------------------------------------------------|-------------------------------------------------------------|
| 50 Mn   |                                                                                        | 900                                                         |
| 50 Cu   |                                                                                        |                                                             |
| 60 Mn   |                                                                                        | 1,140                                                       |
| 40 Cu   |                                                                                        |                                                             |
| 75 Mn   |                                                                                        | 1,140                                                       |
| 25 Cu   |                                                                                        |                                                             |
| 82.5 Mn |                                                                                        | 950                                                         |
| 17.5 Cu |                                                                                        |                                                             |
| 90 Mn   |                                                                                        | 780                                                         |
| 10 Cu   |                                                                                        |                                                             |
| 72 Mn   |                                                                                        |                                                             |
| 18 Cu   |                                                                                        | 1,200                                                       |
| 10 Ni   |                                                                                        |                                                             |

The above described binary and ternary alloys, due to their high coefficient of expansion and high electrical resistance are very useful in the fabrication of thermostatic metals, particularly those thermostatic metals such as bimetal, trimetal and other plural laminae thermostatic metals. In the fabrication of such thermostatic metals a lamina of the above manganese alloy is fused or otherwise bonded to a lamina of a metal or alloy having a low coefficient of expansion such as Invar or nickel-iron alloys containing between 35% and 50% nickel. If desired, the low expansion lamina can be made from a ternary alloy of iron, nickel and titanium. In such case the nickel content will range from 35% to 50%, the titanium content from 1% to 4%, and the remainder iron. The preferred iron-nickel-titanium alloy for the low side contains from 35% to 42% nickel, about 2.5% titanium, and the remainder iron.

One of the best thermostatic bimetals available on the market is known as Chace #2400. The Chace #2400 bimetal has a low side of Invar (36% nickel, balance iron) and a high expanding side of 22% nickel, 3% chromium, balance iron by weight. It is interesting to compare the 2400 thermostatic bimetal with the herein preferred bimetal; namely, that having a low expanding lamina of Invar and a high expanding lamina of 72% manganese, 18% copper, 10% nickel by weight. A very careful and exhaustive study of these two bimetals has been made which shows that the thermostatic metal, which is the subject of this invention, is surprisingly superior to the best of the known bimetals. A summary of this study is set forth below:

| Advantage gained through use<br>of 72% Mn, 18% Cu, 10% Ni<br>and Invar thermostatic bi-<br>metal over #2400 thermostatic<br>bimetal |  | Manner of use                                         |
|-------------------------------------------------------------------------------------------------------------------------------------|--|-------------------------------------------------------|
| 50%<br>1. Strain energy                                                                                                             |  | Constant temperature difference:<br>Identical size.   |
| 58%<br>2. Strain energy                                                                                                             |  | Constant temperature difference:<br>Identical weight. |
| 30%<br>3. Temperature rise                                                                                                          |  | Constant electrical current: Identical<br>size.       |
| 156%<br>4. Strain energy                                                                                                            |  | Constant electrical current: Identical<br>size.       |
| 170%<br>5. Strain energy                                                                                                            |  | Constant electrical current: Identical<br>weight.     |

Strain energy is the force developed by restraining thermal deflection of the bimetal and is the measure of the work which the bimetal can do.

The above summary shows (1) On the basis of a given temperature difference for pieces of the same size, the ratio of the strain energy available through the use of the new manganese thermostatic bimetal and the 2400 bimetal is 1.5 to 1; (2) This relationship, as mentioned immediately above in paragraph (1), for pieces of the same weight of the new manganese thermostatic bimetal and the 2400 bimetal is 1.58 to 1. (3) The fact that the electrical resistivity of the new material is considerably higher than that of the older #2400 results in an added advantage in those cases where the temperature change is accomplished from the passage of electric current. The ratio of the temperature differentials of pieces of the same size of several materials when heated by the passage of the same quantity of electric current will, in the general case where temperature difference is a linear function of heat input, be proportional to the ratio of the electrical resistivity for the materials in question. It follows then that the ratio of the temperature rise of the new thermostatic bimetal to the #2400, when pieces of the same size are heated by the passage of equal amounts of electric current is 1.308 to 1. (4) The ratio of strain energy or work resulting from the passage of equal amounts of electric current through pieces of the same size of the new manganese Invar thermostatic bimetal and the #2400 bimetal is 2.566 to 1. (5) The relationship mentioned directly above in paragraph (4) for pieces of the new manganese Invar thermostatic bimetal and the #2400 bimetal of identical weight is 2.70 to 1.

In the above described bimetal the difference between the coefficients of expansion of the high and low expanding laminae is greater than in those bimetals heretofore known. The advantages of increasing the difference in the expansion

rates of the two laminæ are evident. For example, where such bimetal is used in temperature responsive mechanisms and controls, for a given size of control element the deflection or strength of the element is increased compared with a control element of other known bimetals of such given size, thus making the instrument or device in which it is used more positive or sensitive. Further, because of the high deflection rate and strength of such bimetal, where a given combination of strength and deflection is needed in a control element, smaller amounts can be used than is possible where the control element is made from other known bimetals, thus effecting a saving in the cost of the control element. Since this high electrical resistance bimetal has a higher deflection rate than any other known bimetal, it lends itself to great utility in the manufacture of low amperage circuit breakers.

The thermostatic laminated metal which is the subject matter of this invention gives a greater work output for a given electrical input than those thermostatic laminated metals heretofore known. This is important, particularly in electrical devices where the electrical resistance of the thermostatic metal element is important. In such an electrical device where a thermostatic element having a given electrical resistance and deflection is desired, it is necessary to use a relatively small piece of the heretofore known thermostatic metals. This was disadvantageous because such a small piece of thermostatic metal gave correspondingly small power. On the other hand in such an electrical device, due to the high electrical resistance of the instant thermostatic metal, to satisfy such given electrical resistance and deflection a piece of the instant thermostatic metal can be used which is larger than the usable piece of heretofore known thermostatic metals. Due to the fact that a relatively larger piece of the instant thermostatic metal can be used, such piece of thermostatic metal will give more power.

In the drawings:

Fig. 1 shows the temperature expansion coefficient data of two copper-manganese alloys compared with standard materials.

Fig. 2 shows a bimetal strip having a high expanding lamina of manganese, copper and nickel and a low expanding lamina of Invar. The two laminae are welded together.

Fig. 3 is an illustrative showing of a portion of

a water heater, the burner of which is controlled by a tube and rod type thermostat.

The gas supply is admitted through pipe 1 into valve chamber 2 and passes through pipe 3 into the burner (not shown). The valve housing 2 is provided with a valve 4 pivoted as at 5 and backed up by a compression spring 6 which tends at all times to hold valve 4 in the closed position shown, thereby cutting off the flow of gas through pipe 3 to the burner. The hot water tank is designated 7.

Valve 4 is controlled by a thermostat in the form of a tube 8 secured to the tank 7 as at 9 and a rod 10 mounted within the tube 8 and contacting the tube 8 at 11. Tube 8 is made of the above described high expansion alloy of manganese, copper and nickel. The rod 10 can be any suitable expansion alloy such as Invar. In the position shown, the water in the tank is at the elevated temperature desired. As the temperature of the water in the tank 7 falls, tube 8 will contract thereby raising rod 10 which swings valve 4 about its pivot 5 thereby opening valve 4 and permitting gas to flow through line 3 to the heater. As the temperature of the water rises, rod 8 will expand thereby lowering rod 10 which permits spring 6 to close valve 4 and thereby stop the flow of gas through line 3 to the heater.

We claim:

- Thermostatic metal comprising a plurality of joined metallic laminations, one of said laminations having a relatively high coefficient of expansion and comprising an alloy of the following constituents by weight: manganese from 20% up to 50%, nickel 4% to 20%, balance substantially all copper; the other lamination having a relatively low coefficient of expansion.
- In a device responsive to temperature changes to perform work or mechanical movement, a plurality of metallic members, one of said members having a relatively high linear coefficient of thermal expansion and comprising an alloy of the following constituents by weight: manganese from 20% to 50%, nickel 4% to 20%, balance substantially all copper; the other member having a relatively low linear coefficient of thermal expansion and comprising essentially "Invar," an alloy of iron and nickel.